

[54] PROCESS OF MAKING HIGH STRENGTH,  
HIGH DENSITY, HIGHLY DUCTILE  
URANIUM-TITANIUM ALLOY

[75] Inventors: **Ralph E. Edelman**, Philadelphia,  
Pa.; **Anthony Saia**, Williamstown,  
N.J.

[73] Assignee: **The United States of America as  
represented by the Secretary of the  
Army**, Washington, D.C.

[22] Filed: Oct. 1, 1971

[21] Appl. No.: 185,812

[52] U.S. Cl. .... 148/11.5 F, 102/52, 148/132

[51] Int. Cl. .... C21d 1/18, F42b 11/14

[58] Field of Search ..... 148/132, 11.5 R,  
148/11.5 F, 12.7, 158; 102/52

[56] References Cited

OTHER PUBLICATIONS

Douglass et al., Effect of Heat Treatment on the Hard-

ness and Microstructure of U-Ti Alloys, in *J. Met.*  
9:P. 1260-1267, Oct. 1957.

Primary Examiner—Carl D. Quarforth

Assistant Examiner—R. E. Schafer

Attorney—Harry M. Saragovitz et al.

[57] ABSTRACT

The step of furnace tempering a solution treated, wa-  
ter-quenched, worked cast ingot at 600°F for about 4  
hours in an inert atmosphere and permitting the ingot  
to furnace cool in that atmosphere yields an uranium-  
1.25 titanium alloy having the following physical prop-  
erties:

Tensile strength : 234,700 psi

Yield strength : 172,700 psi

Elongation in 1 inch : 17%

Nominal density : 18.5g/cc

6 Claims, No Drawings

**PROCESS OF MAKING HIGH STRENGTH, HIGH DENSITY, HIGHLY DUCTILE URANIUM-TITANIUM ALLOY**

The invention described herein may be manufactured, used, and licensed by or for the Government for governmental purposes without the payment to us of any royalty thereon.

This invention relates to alloys and more particularly concerns processes for fabricating a high strength, high density, highly ductile uranium-titanium alloy.

Armor-piercing projectiles and the like for modern day munitions must be strong, ductile, and of high density.

Without sufficient ductility, the armor-piercing penetrator might fragment or fracture upon impact with an enemy target. If the target comprises but a single armor layer, fragmenting of the penetrator upon impact therewith might not be unduly detrimental. Where, however, enemy targets comprise spaced armor layers, as in many modern tanks and flying craft, it is imperative that the armor-piercing penetrator remain integral upon impact if successful penetration of the layers is to be achieved.

Furthermore, the armor-piercing projectiles must be sufficiently strong to withstand impact and be of sufficiently high density to render them capable of penetrating these enemy targets. In this regard, prior art armor-piercing penetrators and projectiles do not possess the high strength, high density and high ductility properties required of modern day munitions.

It is therefore an object of this invention to provide an alloy having high strength, high density, and high ductility.

Another object of the invention is to provide such an alloy which would make it ideally suitable for armor-piercing capabilities.

The exact nature of this invention as well as other objects and advantages thereof will be readily apparent from consideration of the specification that follows.

In accordance with the above objects, we have discovered that a uranium base alloy which includes a minor proportion of titanium, will yield a highly ductile

duction furnace at room temperature, the furnace temperature then being brought to about 2,800°F and held at this temperature until the melt is substantially homogeneous.

5 The titanium will preferably comprise 1.25 weight percent of the alloy, but may range from about 1.10 to 1.40 weight percent thereof. If quantities less than about 1.10 weight percent are employed, we have found the resultant alloy to lack sufficient strength for 10 armor-piercing devices. Conversely, when the titanium exceeds about 1.40 weight percent of the alloy, an undesirably brittle piece results.

The melt may now be poured into another mold, suitably magnesia, alundum, thoria, and the like, to form 15 a rod or bar shaped casting of desired dimensions. This cast ingot will now be worked, by extrusion, forging, rolling, etc. and then subjected to a heat treatment as follows:

Solution treat the worked cast ingot at 1650°-1700°F for about 16 hours. The ingot may be placed in the vacuum furnace while maintained at room temperature or at the desired end temperature of 1650°-1700°F.

The solution treated ingot will then be removed from the vacuum furnace and immediately water quenched prior to a tempering treatment which comprises placing the quenched ingot alloy in a furnace maintained at room temperature containing an inert atmosphere, preferably helium. The furnace is brought up to 600°F in about 1 hour, held for 4 more hours, and permitted to cool to about room temperature in about 1-2 hours, the inert atmosphere being maintained throughout. It is this tempering or ageing step which is considered vital in the retention of desired ductility and strength.

More specifically, our melt was cast into ingots having a diameter of 2 1/8" and a length of about 3 inches. These were forged in air at approximately 1650°F into 1/4 inch diameter rods, then hot swaged at approximately 1650°F to 1/2 inch diameter. They were then machined to remove the forged surfaces prior to the heat treatment above described.

Tensile bars were cut from these heat treated bars. The table below lists various mechanical properties of these specimens for our preferred alloy composition.

TABLE I

| High strength, high ductility, high density U-Ti alloy |                 |                                                                                                        |                          |                        |                  |                         |
|--------------------------------------------------------|-----------------|--------------------------------------------------------------------------------------------------------|--------------------------|------------------------|------------------|-------------------------|
| Number                                                 | Alloy           | Heat treatment                                                                                         | Tensile strength, p.s.i. | Yield strength, p.s.i. | Elongation in 1" | Nominal density, g./cc. |
| 1.....                                                 | 98.75U-1.25Ti.. | 1,650-1,700° F.—16 hours in vacuo; water quenched; 600° F.—4 hours (helium); furnace cooled in helium. | 234,700                  | 172,700                | 17%-----         | 18.5                    |
| 2.....                                                 | 98.75U-1.25Ti.. | Same as No. 1, except specimen air cooled instead of furnace cooled..                                  | 200,000                  | 176,000                | 7.2%-----        | 18.5                    |
| 3.....                                                 | 98.75U-1.25Ti.. | Same as No. 2, except water quenched.....                                                              | 154,000                  | -----                  | Broke brittle..  | 18.5                    |

alloy having good strength and density when said alloy is made in accordance with our process steps.

More specifically, we have found that when about 1.25 weight percent titanium is alloyed with the uranium, an alloy can be formed when using our inventive process steps having a tensile strength of 234,700 psi; a yield strength of 172,700 psi; an elongation in 1 inch of 17 percent; and a nominal density of about 18.5g/cc.

In producing our inventive alloy, we place a measured quantity of commercial, high purity (99.9 percent) uranium dingot at the bottom of a crucible, suitably of magnesia or graphite+ceramic-wash, and titanium sponge of commercial purity thereabove, the crucible and contents then being placed in a vacuum in-

55 We wish it to be understood that we do not desire to be limited to the exact details described, for obvious modifications will occur to a person skilled in the art.

We claim:

1. A process for making an armor-piercing munition from a worked cast ingot uranium-titanium binary alloy by increasing strength and ductility of said alloy while providing a high density thereto, said alloy being uranium based and containing about 1.10 to 1.40 weight percent titanium, the steps comprising

60 solution treating said alloy in a vacuum furnace maintained at 1650°-1700°F for a period of about 16 hours, water quenching said solution treated ingot alloy,

tempering said quenched ingot alloy at 600°F for a period of about 4 hours in an inert atmosphere, furnace cooling said tempered ingot alloy in said inert atmosphere, and shaping said cooled tempered ingot alloy into said armor-piercing munition.

2. The process as described in claim 1 wherein said titanium is present in said alloy in an amount of 1.25 weight percent, the balance being substantially uranium, and wherein tensile strength of said alloy is about 234,700 psi, yield strength of said alloy is about 172,700 psi, elongation in 1 inch of said alloy is about 17 percent and nominal density of said alloy is about 18.5g/cc.

3. The process as described in claim 2 wherein said worked ingot comprises the steps of

forging said ingot in air at about 1,650°F, and hot swaging said forged ingot prior to said solution treatment.

4. The process as described in claim 2 further characterized by said inert atmosphere being helium.

5. The process as described in claim 2 further characterized by said tempering step comprising

placing said water quenched ingot in a furnace maintained at room temperature in said inert atmosphere,

raising the temperature of said furnace to about 600°F in a period of about 1 hour while maintaining said inert atmosphere.

6. The process as described in claim 5 further characterized by said inert atmosphere being helium.

\* \* \* \* \*

20

25

30

35

40

45

50

55

60

65